

June 2, 1942.

G. S. FULCHER

2,285,026

CAST REFRACTORY BLOCK

Filed Sept. 23, 1939



*Gordon S. Fulcher*  
Inventor

*Disney Cole & Garner*  
Attorneys

## UNITED STATES PATENT OFFICE

2,285,026

## CAST REFRACTORY BLOCK

Gordon S. Fulcher, Chevy Chase, Md., assignor to  
Corhart Refractories Company, Louisville, Ky.,  
a corporation of Delaware

Application September 23, 1939, Serial No. 296,311

3 Claims. (Cl. 72—39)

In my prior application Serial No. 166,155, filed September 28, 1937, Patent No. 2,201,723, I disclosed a method of producing a cast refractory block from molten material in which the cavities resulting from the contraction of such material during solidification are substantially symmetrical in respect to an axis of the block which was horizontal during the casting and unsymmetrical with an axis which was vertical during the casting, such blocks being shown therein as an L-shaped block which was cast with one limb horizontal and in which the cavities resulting from contraction are segregated at one end of the limb, specifically the free end, by rotating the block in the plane of the said limbs. Such a block has numerous uses in glass tanks and forms the subject matter of this invention.

The accompanying drawing is a perspective view of a block embodying my invention here sought to be protected and in this drawing the block is shown as being substantially L-shaped, consisting of the two limbs *a* and *b* and in which the cavities resulting from contraction are concentrated as at *c* at the free end of the limb *a*.

By casting this block with one of the limbs substantially horizontal a very dense structure is produced in the other limb and by tilting the block around the axis *d*—*d* at right angles to the plane of the limbs of the block, (as shown, by either of the arrows) before the block has solidi-

fied the cavities will be concentrated and segregated in the resultant upper end of the previously horizontal limb, thus producing a solid and dense structure of the block at the junction of the two limbs.

Having thus described my invention what I claim and desire to procure by Letters Patent is:

1. A cast block of refractory material, the cavities resulting from the contraction of such material during solidification being substantially symmetrical in respect to an axis of the block which was horizontal during the casting and substantially unsymmetrical with an axis which was vertical during the casting.
- 15 2. A two-limbed cast block of refractory material, the cavities resulting from the contraction of such material during solidification being segregated at the free end of that limb of the block which was substantially horizontal during the casting.
- 20 3. The hereinbefore described method of casting and solidifying an L-shape refractory block from molten material which comprises positioning a proper mold with one limb vertical and the other horizontal, pouring the molten material into the mold and thereafter during solidification turning the mold around a horizontal axis located near the junction of the two limbs.